

## 1

3,287,149

**REPULPABLE PRINTED PAPER HAVING WATER RESISTANT COATING**

Joseph A. Dooley, Belleville, Richard D. Vieth, Kinnelon, and Harry Burrell, North Caldwell, N.J., assignors to Interchemical Corporation, New York, N.Y., a corporation of Ohio

No Drawing. Filed Jan. 22, 1963, Ser. No. 253,039  
 6 Claims. (Cl. 117—15)

The present invention relates to repulpable coated paper and more particularly to repulpable coated printed paper stock which has sufficient gloss and resistance to water or weathering to be used for magazine covers.

Coated paper used for magazine covers must have the following properties: (1) it must have very high gloss (2) it must be resistant to water since it is generally exposed to weathering (3) it must cure rapidly since in conventional high speed coating operations for magazine covers, the curing time may be as low as a fraction of a second and (4) finally, and most important, the coated stock must be repulpable, that is the coating must be readily removable from the paper by the application of a dilute, about 2%, aqueous sodium hydroxide solution which is used in commercial deinking processes.

As far as it is known to us, no previous coated paper has achieved this unique combination of properties without any attendant properties which are detrimental to the use of the coated paper as a magazine cover. It is indeed rare to find a coated paper which is highly water resistant so that it may withstand the effects of weathering in exposed newsstands, thereby protecting printed matter, and yet may have its coating readily and completely removable by a dilute alkaline solution.

Among coated papers which have been previously tried for magazine covers, thermoset alkyd-amine coated papers have been found to be virtually unrepulpable because the coating can not be separated from the paper and the inks by a dilute alkaline solution. In addition alkyd-amine coatings do not dry at a sufficiently rapid rate to be utilizable in the high speed printing of magazine covers. On the other hand, oleoresinous coatings have been too slow in drying when applied in the film thicknesses required for high gloss in coatings for magazine stock. Furthermore, nitrocellulose lacquer coatings have less than desirable flammability properties and are too low in gloss for use as magazine coatings.

We have now found a novel coated paper which has all of the desirable required properties set forth above for magazine covers without any attendant detrimental properties.

The coated paper of this invention comprises a printed magazine stock substrate coated with a copolymer comprising the copolymerization product of styrene and the half-ester formed by the half-esterification of an alpha-beta unsaturated dicarboxylic acid such as fumaric or maleic acids with a lower alkanol which has 1 to 8 carbons and preferably 1 to 4 carbons, most preferably a n-alkanol such as methanol, n-propanol and n-butanol as well as n-octanol and 2-ethyl hexanol. That this composition may be removed from the paper by treating with a dilute aqueous sodium hydroxide solution is indeed surprising because compounds containing substantial amounts of styrene are conventionally believed to have at least some alkali resistance.

In the present specification and claims, all proportions are by weight unless otherwise stated.

In preparing the copolymers used in the coating the half-ester is first formed by esterifying the alkanol with the alpha-beta unsaturated acid, preferably at a temperature in the range of from 170 to 300° F., after which the half-ester is polymerized, using a conventional addition

## 2

polymerization catalyst, with styrene. During the formation of the half-ester from about 1.1 to 5.0 moles of alkanol are preferably added for each mole of alpha-beta unsaturated acid. During the copolymerization, preferably about from 0.5 to 2.2 moles and most preferably 1 mole of styrene are added for each mole of alpha-beta acid originally present. The copolymerization is preferably conducted at a temperature of from 200 to 350° F.

As will be illustrated in the examples, the coatings on the paper of this invention may be readily removed during conventional repulping or deinking in which the paper is treated with about a 2% solution of sodium hydroxide.

The following examples will illustrate the practice of this invention.

**EXAMPLE 1**
*Copolymer of styrene and butyl-maleic half ester*

|                  |       | Grams |
|------------------|-------|-------|
| Butanol          | ----- | 1836  |
| Maleic anhydride | ----- | 558   |
| Benzoyl peroxide | ----- | 30    |

The above mixture is heated to 210° F. Then 1248 g. of styrene are added slowly over a period of 1 hour while the mixture is maintained at said temperature. Heating is continued until a viscosity of about  $Z_6$  on the Gardner-Holdt Scale is achieved.

**EXAMPLE 2**
*Copolymer of styrene and methyl-maleic half ester*

|                  |       | Grams |
|------------------|-------|-------|
| Methanol         | ----- | 140   |
| Maleic anhydride | ----- | 392   |
| Xylene           | ----- | 624   |
| Benzoyl peroxide | ----- | 25    |

The above mixture is heated to 210° F. Then 460 g. of propanol are added and 832 g. of styrene are added slowly over a period of one hour while the mixture is maintained at 210° F.

**EXAMPLE 3**
*Copolymer of styrene and propyl-maleic half ester*

|                  |       | Grams |
|------------------|-------|-------|
| Propanol         | ----- | 1480  |
| Maleic anhydride | ----- | 558   |
| Benzoyl peroxide | ----- | 30    |

The above mixture is heated to 210° F. Then 1248 g. of styrene are added slowly over a period of one hour while the mixture is maintained at 210° F.

**EXAMPLE 4**

|                  |       | Grams |
|------------------|-------|-------|
| 2-ethyl hexanol  | ----- | 2830  |
| Maleic anhydride | ----- | 558   |
| Benzoyl peroxide | ----- | 30    |

The above mixture is heated to 210° F. Then 1248 g. of styrene are added slowly over a period of one hour while the mixture is maintained at 210° F.

**EXAMPLE 5**

68.9 parts of the copolymer of Example 1 are mixed with 31.1 parts of xylene and the resulting solution is coated by gravure coating onto magazine cover stock at 6 to 8 milligrams per square inch and cured for 0.5 second in a 700° F. air impingement oven. The coated stock displays good block resistance when subjected to 2 lbs./in.<sup>2</sup> pressure for 2 hours at 150° F. as well as excellent gloss and water resistance.

In order to test for repulpability of the coated stock,

about 100 square inches of the stock are shredded and placed in a conventional bath for repulping magazine stock comprising 250 ml. of a 2% aqueous sodium hydroxide solution, to which there has been added 1 g. of 325 mesh mica as a filtering aid and 3 g. of a wetting agent such as the commercial "Vel," sodium dodecylbenzene sulfonate, the bath having a temperature of 140° F. The mixture is stirred vigorously for 15 minutes. The slurry is poured onto a 40 mesh screen and washed with cold tap water. The mixture is reslurried, stirred for several minutes and again washed through a screen as described above. The slurry is then vacuum dried. Careful inspection of the remaining pulp reveals that the coating has completely disintegrated and been removed.

#### EXAMPLE 6

66.7 parts of the copolymer of Example 2 are mixed with 16.7 parts of xylene and 16.6 parts of propanol and the resulting solution is coated by gravure coating onto a magazine cover stock at 6 to 8 milligrams per square inch and cured in an oven at 275° F. for 10 minutes. The coated stock has slightly better block resistance as well as slightly less gloss than the stock of Example 4. The water resistance of the stock is excellent. When tested for repulpability in accordance with the procedure of Example 4, the remaining pulp has substantially no coating adhering to the printed or unprinted surfaces indicating that the coating has been completely disintegrated.

#### EXAMPLE 7

Example 5 is repeated using the same conditions, proportions and ingredients except that 68.9 parts of the copolymer of Example 3 are used. The resulting coated stock has a block resistance slightly better than that of Example 5 but not quite as good as that of Example 6 and a gloss slightly better than that of Example 6 but not quite as good as that of Example 5. The water resistance of the stock is excellent.

When tested for repulpability in accordance with the procedure of Example 5, the remaining pulp has substantially no coating adhering thereto indicating that the coating has been completely disintegrated.

#### EXAMPLE 8

Example 5 is repeated using the same conditions, proportions, and ingredients except 68.9 parts of the copolymer of Example 4 are used. The resulting coated stock has about the same properties as the stock of Example 5. When tested for repulpability in accordance with the procedure of Example 5, the remaining pulp has substantially no coating adhering thereto indicating that the coating has been completely disintegrated.

It should be noted that the magazine stock described 55

in Examples 5 to 8 which is coated may and in commercial practice does contain printed matter. The magazine stock may be printed upon with any conventional ink used in magazine covers e.g., heat-set inks such as inks having limed and zinkated rosin binders and phenolic binders modified with a phenol formaldehyde condensate. All of these conventional inks are readily removed during the repulping process by the action of the dilute alkali. Repulping is also known as deinking.

10 While there have been described what is at present considered to be the preferred embodiments of this invention, it will be obvious to those skilled in the art that various changes and modifications may be made therein without departing from the invention, and it is, therefore, aimed to cover all such changes and modifications as fall within the true spirit and scope of the invention.

What is claimed is:

1. A repulpable coated paper comprising a paper substrate having printing thereon and a water resistant coating over the printing, said coating consisting essentially of the copolymerization product of styrene and the half-ester formed by the half esterification of 1 mole of an alpha-beta unsaturated dicarboxylic acid selected from the group consisting of maleic and fumaric acids with 25 from 1.1 to 5.0 moles of a lower alkanol, from 0.5 to 2.2 moles of styrene being copolymerized for each mole of said acid.
2. The repulpable coated paper of claim 1 wherein said alkanol has from 1 to 4 carbons.
3. The repulpable coated paper of claim 1 wherein said half-ester is the methyl half-ester of maleic acid.
4. The repulpable coated paper of claim 1 wherein said half-ester is the propyl half-ester of maleic acid.
5. The repulpable coated paper of claim 1 wherein said half-ester is the butyl half-ester of maleic acid.
6. The repulpable coated paper of claim 1 wherein said half-ester is the 2-ethyl hexyl half-ester of maleic acid.

#### References Cited by the Examiner

##### UNITED STATES PATENTS

|           |         |                |            |
|-----------|---------|----------------|------------|
| 1,870,358 | 8/1932  | Dils           | 162—8      |
| 1,966,238 | 7/1934  | Drewsen        | 162—8      |
| 2,047,398 | 7/1936  | Voss et al.    | 260—78.5 X |
| 2,254,382 | 9/1941  | Neher          | 260—78.5 X |
| 2,320,724 | 6/1943  | Gerhart et al. | 260—78.5 X |
| 2,576,914 | 12/1951 | Barrett        | 117—155    |
| 2,667,462 | 1/1954  | Wildish et al. | 117—155 X  |
| 3,002,860 | 10/1961 | Bishop et al.  | 117—155    |
| 3,020,178 | 2/1962  | Sweeney et al. | 117—155    |

WILLIAM D. MARTIN, Primary Examiner.

MORRIS O. WOLK, S. L. BASHORE, H. W. MYLIUS,  
Assistant Examiners.

UNITED STATES PATENT OFFICE  
CERTIFICATE OF CORRECTION

Patent No. 3,287,149

November 22, 1966

Joseph A. Dooley et al.

It is hereby certified that error appears in the above numbered patent requiring correction and that the said Letters Patent should read as corrected below.

Column 1, line 71, for "ragne" read -- range --; column 2, line 8, for "350° F." read -- 250° F. --.

Signed and sealed this 12th day of September 1967.

(SEAL)

Attest:

ERNEST W. SWIDER

Attesting Officer

EDWARD J. BRENNER

Commissioner of Patents